

Oct. 24, 1961

G. C. GRAHAM, JR

3,005,456

CATAMENIAL DEVICE

Filed July 3, 1956

Fig. 1.



Fig. 2.



Fig. 3.



INVENTOR  
GEORGE C. GRAHAM JR.

BY  
Alexander T. Kardos  
ATTORNEY

1

3,005,456

## CATAMENIAL DEVICE

George Cooley Graham, Jr., Colonia, N.J., assignor to  
Personal Products Corporation, a corporation of New  
Jersey

Filed July 3, 1956, Ser. No. 595,716  
13 Claims. (Cl. 128—285)

The present invention relates to catamenial devices of improved absorbency and to methods of making the same. More specifically, the present invention is concerned with catamenial napkins and tampons having greater fluid absorptive capacities than are possessed by presently-use cellulosic catamenial devices.

Catamenial devices presently in use depend primarily for their efficiency upon the capacity of their fibrous absorptive pad portions to receive, absorb and retain menstrual fluids. These fibrous pad portions are normally made of cellulosic materials, notably wood pulp, paper, cotton, rayon, or blends and mixtures thereof, which possess excellent absorptive characteristics and properties. Notwithstanding such characteristics and properties, however, the efforts to increase the absorptive capacities of such materials are many and varied.

For example, larger and bulkier tampons and napkins have been manufactured and possess greater absorptive capacities but are not fully acceptable inasmuch as the increased size and volume have caused irritation and discomfort, particularly in the case of catamenial tampons. Other efforts have been directed to the use of more highly compressed catamenial devices by using greater pressures on the fibrous materials during the processing and manufacturing of these sanitary devices whereby greater masses of fibers can be contained within normal or regular sizes and theoretically absorb and hold more fluid. Such efforts, however, have similarly not met with complete success. All in all, a great deal of effort has been expended toward the development of improved absorbent bodies but there still remains considerable room for improvement.

It is therefore a principal object of the present invention to provide a catamenial device of improved absorbency without necessarily requiring greater amounts of absorbent fibrous materials or the use of greater pressures during the manufacturing of such devices.

It has been found that the use of a modified cellulosic product, namely a carboxylalkyl cellulose salt, such as sodium carboxymethyl cellulose or sodium carboxyethyl cellulose, in such catamenial devices creates enhanced fluid absorptive capacities therein, provided the average degree of substitution of the carboxylalkyl radical in the cellulose molecule is maintained within controlled limits and is not permitted to exceed specified values to be described more fully hereinafter.

In the accompanying drawings and following specification, there are illustrated and described preferred designs of articles of manufacture embodying the present invention, but it is to be understood that the inventive concept is not to be considered limited to the constructions disclosed except as determined by the scope of the appended claims.

Referring to the accompanying drawing:

FIG. 1 is a cross-sectional view of a sanitary napkin, containing the improved absorbent pad of the present invention;

FIG. 2 is a cut-away view in elevation of a catamenial tampon containing an improved absorbent pad of the present invention; and

FIG. 3 is a graph showing the fluid absorptive capacities of a carboxymethyl cellulose tampon of the present invention.

2

In the embodiments of the invention shown in the drawing, a sanitary napkin 1 comprises an upper fibrous absorptive pad 2 and a lower fibrous absorptive pad 3 (both preferably of fluffed wood pulp) which are separated by a water repellent tissue layer 4. Both pads 2, 3 and the layer 4 are folded within an envelope 5 made of paper or similar material, which, in turn, is wrapped within an external textile cover 6 of a non-woven material or of a woven material such as gauze.

10 The textile cover 6 has a length greater than the other elements above-recited and extends beyond the ends thereof to form fastening or pinning tabs (not shown) to position the napkin in place to conform to the body contours of the user and to receive, absorb and retain catamenial fluids. This structure is exemplary of a form of sanitary napkin in commercial use and is employed to illustrate the invention. It should be realized, however, that such is not to be construed as limitative of the broader aspects of the present invention.

15 20 In FIG. 2, there is illustrated a catamenial device 10 comprising a hollow cylindrically-shaped container or applicator 11 and a smaller plunger or ejector 12, slidably positioned within the applicator 11. A fibrous absorptive pad 13 (preferably of cotton or cotton and other cellulosic materials) is positioned within the applicator 11 and is adapted to be slidably ejectible therefrom by movement of the plunger 12 into the applicator 11 so as to be positioned in a body cavity to conform to the body contours of the user and to receive, absorb and retain catamenial fluids. A withdrawal string or cord 14 is secured preferably to the base of the tampon and is of sufficient length that the free end thereof extends outwardly of the body cavity for withdrawal of the tampon after use. This structure, similarly, is exemplary of a form of catamenial tampon in commercial use and is employed primarily to illustrate the invention. It should be realized, however, that such is not limitative but merely illustrative of the invention.

25 30 35 40 45 50 55 The fibrous absorptive pad portions 2 and 3 of the sanitary napkin 1 are normally manufactured from a fluffed cellulosic wood pulp product wherein the average lengths of the cellulosic fibers are relatively short, usually less than  $\frac{1}{2}$  inch, and are not capable of being processed by standard textile equipment, such as a card. On the other hand, the fibrous absorptive pad portion 13 of the tampon 10 comprises absorbent cellulosic fibers having an average fiber length of at least about  $\frac{1}{2}$  inch and up to about  $2\frac{1}{2}$  inches or longer and are capable of being processed by standard textile equipment (such as a card) into the desired forms and shapes.

55 60 65 70 The cellulosic fibers of these fibrous absorptive pad portions are modified according to the present inventive concept within pre-determined limits whereby their fluid absorptive capacities are considerably enhanced. More explicitly, a specified percentage or proportion of the hydroxyl radicals of the cellulose molecule are modified by etherification or carboxyalkylation processes whereby there is obtained a carboxylalkyl cellulosic product having a calculated degree of carboxylalkyl substitution. These products are exemplified by sodium carboxymethyl cellulose and sodium carboxyethyl cellulose.

In the specification terminology, the term carboxymethyl cellulose (or cellulose glycolic acid ether) refers to the salts thereof, particularly the sodium salt. Similarly, carboxyethyl cellulose (or cellulose hydroxypropionic acid ether) refers to its salts, particularly the sodium salt.

70 The salt of cellulose glycolic acid ether (salt of carboxymethyl cellulose), which may be used to prepare

the catamenial devices of the invention may be described structurally as:



where  $x$  is at least equal to 0.03 but not greater than 0.35 and  $y$  is a large whole number.

The ring structure represents the anhydroglucose residue which is linked in known manner to similar residues on either side to form a long chain cellulose structure. The bracketed H atoms are attached to side-chain oxygen atoms in the anhydroglucose residue in known fashion. Similarly, the bracketed  $-(CH_2-COONa)_x$  groups are attached to the residue through side-chain oxygen linkages by substituting for the aforementioned H atoms.

The salt of carboxyethyl cellulose (salt of cellulose hydroxypropionic acid ether), which is an alternate to the salt of carboxymethyl cellulose, may be described structurally as:



$x$ , again, being at least equal to 0.03 but not greater than 0.35 and  $y$  a large whole number. The  $C_2H_4$  group is preferably  $-\text{CH}_2-\text{CH}_2-$ .

The general formula of the materials used to prepare catamenial devices according to the invention is therefore:



where  $x$  is at least equal to 0.03 but not greater than 0.35,  $n$  is 1 or 2, and  $y$  is a large whole number.

The degree of substitution (D.S.), a term commonly employed in connection with cellulose derivatives of the nature used in the invention catamenial devices, is an important property and indicates the average number of substituent groups per glucose unit in the cellulose molecular chain (i.e., the value of  $x$  in the above formulae). Since there are originally three hydroxyl groups and hence three possible points of substitution per glucose unit, the maximum degree of substitution is 3. It has been found according to the present invention that the degree of substitution is an important factor in determining the absorptive activity of the particular cellulose ether. More specifically, it has been found that, as the degree of substitution increases, the catamenial absorptive capacity also increases up to a maximum but then rapidly falls thereafter off to very low values.

Without being bound to the following theory, it is believed that the increased absorbency is due to the reception and retention of fluids within the individual modified cellulosic fibers in addition to the usual reception and retention of fluids in the capillary spaces between the individual fibers. This phenomenon apparently exists up to a degree of substitution of about 0.35 (approximately one carboxyalkyl radical for every three glucose residues) and surprisingly falls off and dis-

pears when the degree of substitution is increased thereafter.

The graph shown in FIG. 3 illustrates clearly the striking relationship of the degree of substitution and the fluid absorptive capacity of the resulting tampon. The curve shown in FIG. 3 is based on the following table.

Table 1

| Degree of substitution (CMC): | Fluid absorbed tampon wt. |
|-------------------------------|---------------------------|
| 0.05                          | 3.12                      |
| 0.10                          | 4.26                      |
| 0.20                          | 4.28                      |
| 0.27                          | 4.33                      |
| 0.32                          | 2.02                      |

It is quite apparent from the graph that values as low as about 0.03 carboxymethyl substitution show improved results but that values in excess of about 0.35 carboxymethyl substitution markedly decrease the absorptive properties of the materials and consequently render the same undesirable for use in catamenial devices. The tampons used in deriving the values of the above table are the so-called "Super" size, weighing approximately 54 grains (3.5 grams) and having a length of about 25  $1\frac{1}{4}$  inches and a diameter just under 0.6 inch.

The test procedures used in obtaining the values shown in Table 1 are as follows:

The test tampons (dry) comprising carboxymethyl cellulosic fibers having an average fiber length greater than 30  $\frac{1}{2}$  inch are measured for length, diameter and weight and are then placed in porous plate Buchner funnels. A resilient rubber surface which snugly fits within the funnel is lowered to contact the tampon and pressure equal to about 24 inches of water is applied to the tampon 35 through the resilient rubber surface. The test fluid (sp. gr. 1.04) is introduced upwardly through the stem of the funnel and just covers the test tampon. Absorption is permitted to take place at the 24 inch water pressure for 5 minutes. The test fluid is then removed and the 40 test tampon is permitted to drain for 1 minute under the 24 inch water pressure. The pressure is then removed and the wet tampon is removed, quickly weighed and the results recorded. Test samples of similar length, diameter and weight tampons of untreated cotton fibers 45 (0% CMC) are tested along with the 5 and 10% carboxymethyl cellulose test tampons and give comparative results of 2.8 and 2.8, as compared to the 3.12 and 4.26 values obtained for the treated test tampons as noted in the table.

50 The particular process used to introduce the carboxyalkyl radical into the glucose residue in the cellulose may be selected from any of the known processes now used commercially involving the use of cellulose (preferably cotton or fluffed wood pulp in the desired fiber length 55 form), monochloracetic acid and sodium hydroxide. In the case of the fluffed wood pulp, the only requisite is the introduction of the pre-determined number of carboxymethyl radicals in the glucose residues. In the case of the cotton fibers, however, an additional requirement in the selection of the particular process is the control and ability to introduce up to about 0.35 carboxyalkyl groups per glucose residues in the cellulose without destroying the fibrous structure of the cellulosic materials or reducing the fiber length to less than about  $\frac{1}{2}$  inch. 60 The products of such processes are available commercially.

65 It is to be appreciated that, since there is an overall average of less than one carboxyalkyl group per glucose residue, some residues will be unaffected and have no carboxyalkyl groups, whereas others may have one, two or perhaps even three carboxyalkyl groups.

70 Additionally, it is not necessary that all of the fibers be exposed to carboxyalkylating treatment inasmuch as it is possible to carboxyalkylate some of the fibers to higher degrees and then mix, blend, or form layers of

the modified fibers with unmodified fibers whereby the necessary over-all average of below about 0.35 substitution is obtained. Blends of 10-90% cotton and 90-10% modified cotton are found particularly advantageous.

Alternatively, it is possible to carboxyalkylate some of the fibers as high as 0.35 or even to higher degrees and use such fibers in a body as one of the components of an absorptive pad portion, the other components being, for example, lesser modified cellulosic fibers, unmodified cellulosic fibers or other cellulosic materials. In such a case although the degree of carboxyalkyl substitution of the fibers in one component may thus be very high, the over-all average degree of substitution of the complete absorptive pad portion, when you consider all cellulosic components thereof, may be very low and on the order of 0.22, 0.01 or even lower.

As an example of the blending of unmodified cotton and modified cotton, a 50-50 blend (by weight) of 0.32 D.S. carboxymethyl cellulose and unmodified cotton is employed to make a "Super" tampon having physical dimensions as described previously. Such a tampon, when evaluated by the test procedures disclosed herein, possesses a ratio of fluid absorbed to tampon weight of 4.53.

Additional 50-50 blends (by weight) of 0.30 D.S. carboxymethyl cellulose and unmodified cotton, when manufactured into test tampons and evaluated by the test procedures described herein, yield ratios of fluid absorbed to tampon weights of 4.46, 4.69 and 5.05, for samples having densities of 170, 100 and 85 grains per cubic inch respectively. Similar samples of 100% unmodified cotton manufactured to similar specifications yield ratios of fluid absorbed to tampon weight of 2.6, 3.4 and 3.8, respectively.

Although the present invention has been described primarily with carboxymethyl cellulose, it is to be appreciated that carboxyethyl cellulose, such as obtainable from the treatment of the cellulose fibers with sodium hydroxide and monochloropropionic acid, instead of monochloracetic acid, is also applicable within the more general aspects of the present invention.

If desired, the modified cellulosic fibers, either by themselves or in blends or layers with unmodified cellulosic fibers, may be mixed with other fibers to obtain special characteristics and properties. Such other fibers include rayon (regenerated cellulose), cellulose esters (cellulose acetate), vinyl fibers ("Vinyon"), acrylic fibers ("Orlon," "Acrlan"), vinyl-acrylic fibers ("Dyneil"), nylon, saran and "Dacron" polyester fibers. It is to be noted that such fibers, if they are to be used in sanitary napkins in conjunction with fluffed wood pulp, may be very short. On the other hand, if such fibers are to be used in tampons in conjunction with cotton staple of greater length, they should have an average length of at least about  $\frac{1}{2}$  inch so that they will be capable of being processed on standard textile apparatus and equipment.

While I have shown and described what I believe to be a preferred embodiment of the invention in the matter of simplicity of construction, ease of utilization, etc., it will be appreciated that the details of such construction may be more or less modified within the scope of the claims without departure from the principles of construction or material sacrifice of the advantages of the preferred design.

I claim:

1. A catamenial device of improved fluid absorbency comprising a self-supporting, disposable body of absorbent cellulosic fibers having an average degree of sodium carboxyalkyl substitution of not more than about 0.35 carboxyalkyl radicals per glucose residue in the cellulose, said substituted cellulosic fibers being substantially insoluble in water; and means to position said body of

fibers for the reception, absorption and retention of catamenial fluids.

2. A catamenial device as defined in claim 1 wherein the carboxyalkyl radical is carboxymethyl.
3. A catamenial device as defined in claim 1 wherein the carboxyalkyl radical is carboxyethyl.
4. A catamenial device as defined in claim 1 wherein the cellulosic fibers are cotton.
5. A catamenial device as defined in claim 1 wherein the cellulosic fibers are fluffed wood pulp.
- 15 6. A catamenial device of improved fluid absorbency comprising a self-supporting, disposable body of absorbent cellulosic fibers having an average degree of carboxyalkyl substitution of from about 0.03 to about 0.35 carboxyalkyl radicals per glucose residue in the cellulose; and means to position said body of fibers for the reception, absorption and retention of catamenial fluids.
- 20 7. A catamenial device of improved fluid absorbency comprising a self-supporting, disposable body of absorbent cellulosic fibers having an average fiber length of about  $\frac{1}{2}$  inch to about 2 $\frac{1}{2}$  inches, said cellulosic fibers having an average degree of sodium carboxyalkyl substitution of from about 0.03 to about 0.35 carboxyalkyl radicals per glucose residue in the cellulose; and means to position said body of fibers for said reception, absorption and retention of catamenial fluids.
- 25 8. A catamenial device of improved fluid absorbency comprising a self-supporting, disposable, substantially cylindrical body of absorbent cellulosic fibers having an average fiber length of at least about  $\frac{1}{2}$  inch, said cellulosic fibers having an average degree of sodium carboxyalkyl substitution of from about 0.03 to about 0.35 carboxyalkyl radicals per glucose residue in the cellulose; an applicator for containing said cylindrical body of cellulosic fibers; and a plunger to eject said cylindrical body of fibers from said applicator and position the same in a body cavity for use therein as a tampon.
- 30 9. A catamenial device of improved fluid absorbency comprising a self-supporting, disposable, substantially cylindrical body of absorbent cellulosic fibers having an average fiber length of from about  $\frac{1}{2}$  inch to about 2 $\frac{1}{2}$  inches, said cellulosic fibers having an average degree of substitution of from about 0.03 to about 0.35 sodium carboxyalkyl radicals per glucose residue in the cellulose; an applicator for containing said cylindrical body of cellulosic fibers; and a plunger to eject said cylindrical body of fibers from said applicator and position the same in a body cavity for use therein as a tampon.
- 35 10. A catamenial tampon comprising an elongated mass of cellulosic absorbent material adapted to be carried in the vagina of a woman during periods of menstrual discharge and means attached to said mass of cellulosic absorbent material for removing said mass from the vagina, said cellulosic absorbent material containing as an essential ingredient (sodium) carboxymethylcellulose which is fibrous in nature, having an average degree of carboxyalkyl substitution of from about 0.05 to 0.3 carboxyalkyl radicals per glucose residue in the cellulosic material.
- 40 11. A catamenial tampon comprising an elongated mass of absorbent material adapted to be carried in the vagina of a woman during periods of menstrual discharge and means attached to said mass of absorbent material for removing said mass from the vagina, said absorbent material containing as an essential ingredient sodium carboxymethylcellulose which is fibrous in nature and substantially insoluble in water.
- 45 12. A catamenial tampon comprising an elongated mass of absorbent material adapted to be carried in the vagina of a woman during periods of menstrual discharge and means attached to said mass of absorbent material for removing said mass from the vagina, said absorbent material consisting essentially of sodium carboxymethyl-

cellulose which is fibrous in nature and substantially insoluble in water.

13. A catamenial tampon comprising an elongated mass of absorbent material adapted to be carried in the vagina of a woman during periods of menstrual discharge and means attached to said mass of absorbent material for removing said mass from the vagina, said absorbent material consisting primarily of a mixture of substantially, water-insoluble fibrous sodium carboxymethylcellulose and long-fibered cotton.

**References Cited in the file of this patent**

**UNITED STATES PATENTS**

1,736,714 Lilienfeld ----- Nov. 19, 1929 15

|           |                      |               |
|-----------|----------------------|---------------|
| 2,024,218 | Haas -----           | Dec. 17, 1935 |
| 2,486,805 | Seymour et al. ----- | Nov. 1, 1949  |
| 2,626,214 | Osborne -----        | Jan. 20, 1953 |
| 2,773,000 | Masci et al. -----   | Dec. 4, 1956  |

**OTHER REFERENCES**

The Chemical and Physical Properties of Carboxymethylcellulose and its Salts, by Brown and Houghton, from pages 254-258 of October 1941, Soc. Chemical Industrial Journal, Vol. 59, 60, 260-231.

Hollabaugh et al.: Industrial and Engineering Chemistry, Vol. 37, No. 10, October 1945, pages 943-7. (Copy in Division 63, class 260-231.)

UNITED STATES PATENT OFFICE  
CERTIFICATE OF CORRECTION

Patent No. 3,005,456

October 24, 1961

George Cooley Graham, Jr.

It is hereby certified that error appears in the above numbered patent requiring correction and that the said Letters Patent should read as corrected below.

Column 5, line 17, for "0.22" read -- 0.02 --; line 61, for "utilization" read -- utilization --; column 6, line 55, for "cellulosis" read -- cellulosic --.

Signed and sealed this 10th day of April 1962.

(SEAL)

Attest:

ERNEST W. SWIDER

Attesting Officer

DAVID L. LADD

Commissioner of Patents